

## UNITED STATES PATENT OFFICE

ERNEST A. YOUNG, OF SAN ANTONIO, TEXAS, ASSIGNOR TO UVALDE ROCK ASPHALT COMPANY, OF SAN ANTONIO, TEXAS, A CORPORATION OF TEXAS

## NONSKID PAVING SURFACE CONSTRUCTION

No Drawing.

Application filed July 28, 1927. Serial No. 209,179.

This invention relates to a new and improved paving construction and more particularly to a pavement which is provided with means for preventing skidding and giving a firm traction surface.

In its specific form my invention relates to a pavement, the body of which is formed of rock asphalt such as the material known as Uvalde rock asphalt found in natural deposits in Uvalde County, Texas, although other generally similar materials may be used. This Uvalde rock asphalt consists of a comparatively porous shell limestone impregnated naturally with asphalt which fills the pores in the rock. The rock asphalt is comparatively soft when considered relative to trap rock or other hard rocks used for road making.

The Uvalde rock asphalt is commonly used for making roads or other similar surfaces by crushing and grading it and then treating it with a flux such as an asphaltic oil or a paraffine base oil. In some methods of preparation the rock is heated, while by other methods the mixture is made with the materials cold. In some cases a solvent such as kerosene is also added to delay the setting of the mixture, this being more generally used with the cold mixed material. This rock asphalt when so treated, is spread out on a suitable base and compacted by means of a road roller or the like. When so treated a dense smooth surface is formed which is substantially impervious to water and which is very wear-resisting under normal road traffic. Such a surface, however, at times becomes quite slippery when wet or when an excess of the flux is brought to the surface by heat. On steep slopes this surface does not afford adequate traction under such conditions.

It is an object of the present invention to provide a new and improved pavement and method of laying the same which affords an adequate traction effect under all conditions.

It is a further object to provide such a road surface, the base of which is rock asphalt or the like, and which may be commercially produced by usual methods.

It is an additional object to provide a construction of this character in which the traction effect is provided by means of an appli-

cation of crushed stone or the like harder than the rock asphalt base.

Other and further objects will appear as the description proceeds.

According to the present invention rock asphalt may be made into a suitable road forming mix by any one of the methods well known in the art. When so treated the asphalt is laid upon the prepared base and spread in a substantially uniform layer or in such a layer as to give a substantially smooth surface when compacted. It will be understood that this rock asphalt mix when so laid is substantially balanced as to size; that is, the larger and smaller particles are so sized and proportioned as to provide a minimum of voids. After this material is spread a layer of crushed stone is scattered over the first layer of rock asphalt. This crushed stone is preferably considerably harder than the rock asphalt so that it tends to crush the asphalt when forced into it by the compacting roller. The crushed rock is also preferably not balanced as to size and in the preferred construction the crushed rock is substantially a one-sized material. A satisfactory size for the crushed rock has been found to be substantially the size of the coarser rock asphalt aggregate in the rock asphalt layer. After the crushed rock has been scattered the entire mass is thoroughly compacted by means of a road roller or the like.

Under some circumstances it may be found advisable to coat the crushed stone with fluid asphaltic material or with the same material which is used as a flux in forming the rock asphalt base. This coating enables the crushed rock to be more quickly consolidated into an integral mass with the rock asphalt, particularly if the rock asphalt mix has little excess asphaltic material.

It will be understood that the specific details given are by way of illustration only as various types of material may be used as a base and different sizes and kinds of non-skid surface material may be used. I contemplate such changes and modifications as come within the spirit and scope of the appended claims.

55

60

65

70

75

80

85

90

95

100

I claim:

1. The method of laying a pavement or the like which comprises spreading a loose layer of crushed asphalt rock, said rock being sized and proportioned to give a balanced mixture with a minimum of voids, spreading on said first layer a scattered layer of crushed stone harder than the first layer and compacting the layers together.
10. 2. The method of laying a pavement or the like which comprises spreading a loose layer of crushed asphalt rock, said rock being sized and proportioned to give a balanced mixture with a minimum of voids, spreading on said first layer a scattered layer of crushed stone harder than the first layer, said crushed stone being a one-sized aggregate substantially the size of the coarser rock asphalt aggregate, and compacting the layers together.
20. 3. The method of laying a pavement or the like which comprises spreading a loose layer of crushed asphalt rock, spreading on said first layer a layer of crushed stone harder than the first layer, said crushed stone having been coated with a relatively fluid asphaltic material, and compacting the layers together.
30. 4. The method of laying a pavement or the like which comprises spreading a loose layer of crushed asphalt rock, said rock being sized and proportioned to give a balanced mixture with a minimum of voids, spreading on said first layer a scattered layer of crushed stone harder than the first layer, said crushed stone being a one-sized aggregate substantially the size of the coarser rock asphalt aggregate, and being coated with fluid asphaltic material and compacting the layers together.
40. 5. The method of laying a pavement or the like which comprises spreading a loose layer of crushed rock asphalt mixed with a flux, spreading on said first layer a layer of crushed stone harder than the first layer and compacting the layers together.
45. 6. The method of laying a pavement or the like which comprises spreading a loose layer of crushed rock asphalt mixed with a flux, spreading on said first layer a layer of crushed stone harder than the first layer and compacting the layers together, said crushed stone having been treated with the same flux as the rock asphalt.
55. 7. The method of laying a pavement or the like which comprises spreading a loose layer of crushed rock asphalt mixed with a flux, said rock being sized and proportioned to give a balanced mixture with a minimum of voids, spreading on said first layer a layer of crushed stone harder than the first layer and compacting the layers together.
60. 8. A non-skid pavement construction comprising a compacted body of crushed rock asphalt balanced as to size and with a minimum of voids and scattered crushed rock harder than the asphalt rock embedded in the upper surface of the body.

9. A non-skid pavement construction comprising a compacted body of crushed rock asphalt and a flux and scattered crushed rock harder than the asphalt rock embedded in the upper surface of the body and adhering to the rock asphalt body by means of the flux and the asphalt. 70

Signed at San Antonio, Texas, this 2nd day of July, 1927.

ERNEST A. YOUNG.

75